

# UNITED STATES PATENT OFFICE.

RICHARD HERZ, OF FRANKFORT-ON-THE-MAIN, GERMANY, ASSIGNOR TO CASSELLA COLOR COMPANY, A CORPORATION OF NEW YORK.

## PRODUCING FAST DYEINGS ON THE FIBER.

1,107,164.

Specification of Letters Patent.

Patented Aug. 11, 1914.

No Drawing.

Application filed February 21, 1913. Serial No. 749,845.

*To all whom it may concern:*

Be it known that I, RICHARD HERZ, Ph. D., a subject of the King of Prussia, and a resident of Eysseneckstrasse 17, Frankfort-on-the-Main, Germany, have invented certain new and useful Improvements in Producing Fast Dyeings on the Fiber, of which the following is a full description.

I have found that amino—and alkylamino—compounds of carbazole and of its (N-)substituted derivatives may be employed for developing dyeings diazotized on the fiber. The polyamino compounds, particularly the tetraamino compounds of carbazole and of its (N-)substituted derivatives are especially suitable for this process, and the shades so produced are distinguished by exceptionally good fastness to light. The material is dyed or padded in the customary manner with diazotizable colors, or with compounds possessing free amino groups, which colors or compounds are subsequently diazotized and developed with the solutions of the above-named derivatives of carbazole.

25 The method of production is illustrated by the following examples:

Example I: Dye in the customary manner with 4% primulin (see *Farbstofftabellen* by G. Schultz, 5th edition, page 211, No. 616), 30 rinse, diazotize, and develop in a bath containing a weight of the hydrochlorid of tetraaminocarbazole equal to  $\frac{1}{2}$  to 1% of the weight of the goods. In order to neutralize the free mineral acid, a small quantity of soda or sodium acetate may be added to the developing bath. The dyeings are rinsed and dried; by this method deep brown shades are obtained, possessing extreme fastness to washing. If in the place of the 40 tetraaminocarbazole, the tetraamino (N)-ethylcarbazole is used as a developer, the dyeing has a fast purplish brown color, whereas monoamino- and diaminocarbazoles yield with diazotized primulin more olive-brown, mono- and diamino (N) ethylcarbazole yellowish olive shades.

Example II: Dye in the customary manner with 5% diaminogene (see *Farbstofftabellen* by G. Schultz, 5th edition, page 92, 50 No. 274,) extra, diazotize, rinse, and develop as described above with the hydrochlorid of tetraaminocarbazole, rinse, soap with 5 grams soap per liter for about 3 minutes at 40-50° C., rinse again, and dry. In this case of very good fastness

to washing and exceedingly good fastness to light is obtained. The same result is obtained by developing with the hydrochlorid of tetra-amino (N)-methyl carbazole, while mono- and diaminocarbazole yield somewhat 60 more steel blue shades.

Example III: Dye in the customary manner with 4% oxy diamin violet BF (see *Farbstofftabellen* by G. Schultz, 5th edition, page 107, No. 326), diazotize, rinse, and develop in a bath containing a weight of the hydrochlorid of 1. amino-carbazole equal to  $\frac{1}{2}$  to 1% of the weight of the goods. The dyeings are then rinsed, soaped, and dried as described in the above example. Violet 70 shades of very good fastness to milling are thus produced. When substituting for the 1. aminocarbazole the tetra-amino-carbazole or tetra-amino(N) alkylcarbazole, blackish violet shades, and when using diaminocarbazoles, reddish violet shades of the same fastness are obtained.

Example IV: Dye in the customary manner with 4% diamin azo scarlet 4B (see *Farbstofftabellen* by G. Schultz, 5th edition, 80 page 383,) diazotize, rinse, and develop with the hydrochlorid of tetra-amino(N)ethylcarbazole; brick red shades result having good fastness to washing.

Example V: Dye with 6-8% diazo light 85 yellow G (see *Farbstofftabellen* by G. Schultz, 5th edition, page 386,) rinse and diazotize. If developing with the hydrochlorid of tetraaminocarbazole, brown shades, while if developing with tetra-amino(N)ethylcarbazole, red brown shades of excellent fastness 90 to washing and light are formed.

Having now particularly described and ascertained the nature of my said invention, and in what manner the same is to be performed, I declare that what I claim is:—

1. The process for producing fast dyeings on the fiber which consists in developing diazotizable coloring matters on the fiber by coupling the diazotized coloring matters with 100 amino-derivatives of a carbazole compound, substantially as described.

2. The process for producing fast dyeings on the fiber which consists in developing diazotizable coloring matters on the fiber by 105 coupling the diazotized coloring matters with amino-derivatives of (N) substituted carbazole compounds, substantially as described.

3. The process for producing fast dyeings on the fiber which consists in developing 110

diazotizable coloring matters on the fiber by coupling the diazotized coloring matters with tetraamino derivatives of a carbazole compound, substantially as described.

5 4. The process for producing fast dyeings on the fiber which consists in developing diazotizable coloring matters on the fiber by coupling the diazotized coloring matters with tetraamino derivatives of (N) substituted

carbazole compounds, substantially as de- 10  
scribed.

In witness whereof I have hereunto signed my name this 6th day of Feb. 1913, in the presence of two subscribing witnesses.

RICHARD HERZ.

Witnesses:

JEAN GRUND,  
CARL GRUND.

Copies of this patent may be obtained for five cents each, by addressing the "Commissioner of Patents,  
Washington, D. C."